

April 23, 1935.

C. W. MANSUR

1,998,964

METHOD OF MANUFACTURING NONMETALLIC GEAR WHEEL BLANKS AND THE LIKE

Filed May 21, 1930

2 Sheets-Sheet 1



Inventor:  
Clarence W. Mansur,  
by *Charles E. Tullor*  
His Attorney.

April 23, 1935.

C. W. MANSUR

1,998,964

METHOD OF MANUFACTURING NONMETALLIC GEAR WHEEL BLANKS AND THE LIKE

Filed May 21, 1930

2 Sheets-Sheet 2

Fig. 6.



Fig. 8.



Fig. 7.



Fig. 9.



Inventor:

Clarence W. Mansur,  
by Charles E. Tullar  
His Attorney.

## UNITED STATES PATENT OFFICE

1,998,964

## METHOD OF MANUFACTURING NONMETALLIC GEAR WHEEL BLANKS AND THE LIKE

Clarence W. Mansur, Malden, Mass., assignor to  
General Electric Company, a corporation of  
New York

Application May 21, 1930, Serial No. 454,464

4 Claims. (Cl. 154—2)

The present invention relates to the manufacture of bodies such as gear wheel blanks and the like, from a number of dissimilar elements formed from spinnable textile fibers treated with an uncured adhesive, such as a phenolic condensation product which is converted into its hard infusible state upon the application of heat and pressure.

The object of my invention is to provide an improved method of manufacturing such bodies, the advantages of which are pointed out herein-after, and for a consideration of what I believe to be novel and my invention, attention is directed to the following specification and to the claims appended thereto.

15 My improved method is especially well adapted for use in the manufacture of blanks for non-metallic gear wheels, and accordingly I have chosen to illustrate and describe the method as applied to this use. It is to be understood, however, that the invention is not limited thereto necessarily.

20 In the drawings, Figs. 1, 2, 3 and 4 are sectional views illustrating steps utilized in carrying out my invention; Fig. 5 is a perspective view of a completed gear wheel blank made in accordance with the method; Figs. 6, 7 and 8 are sectional views similar to Figs. 1 to 4 illustrating a modification of the invention, and Fig. 9 is a perspective view of a completed gear wheel blank made in accordance with the modified method illustrated in Figs. 6 to 8.

25 In Figs. 1 to 4 I have shown my improved method applied to the manufacture of a non-metallic gear wheel blank wherein the blank is formed from a number of pieces of woven textile material previously treated with an adhesive and cut to provide parts for forming the hub, web and rim of the blank. According to my invention, I provide an annular metal container 1 formed of 30 relatively thin material so that it is light and easy to handle and provided preferably with a number of spaced openings 2 for the admission of steam or hot gases to the interior of the container. The container 1 is open at both ends 35 and is of a diameter corresponding to that of the gear wheel blank to be made. For use with the container 1 I provide a supporting ring 3 which may be made of any suitable material and which fits loosely in the bottom of the container.

40 In carrying out my invention, I first place a container 1 with a ring 3 in the bottom thereof on a support or table 4, and I assemble in the container 1 the several dissimilar elements which are to be utilized in forming the gear wheel blank. In the present instance the elements are

5 shown as comprising pre-formed end sheets 5, intermediate sheets 6, rings 7 which form a part of the rim of the blank and a filling member 8 which forms the thickened portion of the hub. It is to be understood that the elements which go to make up the gear wheel blank illustrated are shown only by way of example and are to be taken as typical of any suitable elements which are to be utilized in the manufacture of the gear wheel. The container 1 is of a size such that the 10 several elements fit in it with sufficient tightness that they are readily held therein. The ring 3 serves simply to keep the parts from being assembled in contact with the support 4 and so that they are held spaced from the lower end of the 15 container.

20 After the elements are assembled in the container 1, the container is placed in a suitable heating oven and heated, the oven preferably containing a moist atmosphere. For this purpose I may heat the elements by means of steam, the steam providing the moist atmosphere, or I may utilize with advantage an electrically heated oven, the moist atmosphere being obtained by injecting steam into the oven. The arrangement 25 may be such that the container passes through the oven on an endless carrier entering at an admission opening and coming out at a discharge opening. I have found that heating for a time of the order of six minutes and at a temperature 30 of the order of 100° to 150° C. satisfactory. By heating the material in this way and preferably in the presence of a moist atmosphere, the adhesive is rendered plastic enough to stick the 35 elements together without, however, curing to any great extent the adhesive and without its becoming sticky enough to stick to a mold.

40 I consider the heating of the material in a moist atmosphere as being one important feature of my invention for by so heating the material I find that a uniform temperature throughout the mass is obtained and that the presence of the moisture prevents the material from sticking to the mold used in making the preform.

45 After the preliminary heating, the container 1 with the elements therein is lifted off the ring 3 and placed in a forming mold and pressed 50 therein to produce a preform. By a preform I mean a body having the general shape of the finished gear wheel blank and stuck together so that it can be handled as a unit, the resin however not being cured to any appreciable extent. The adhesive serves to stick the elements together and hold them. For this initial pressing operation I have found a pressure of the order of 2,000 55

pounds per square inch satisfactory. In Figs. 2 and 3, 9 indicates the outer wall or shell of the forming mold, 10 indicates the lower mold member, the upper surface of which is shaped as is indicated at 11 to the correct contour for forming the blank, and 12 indicates the upper mold member, the lower face 13 of which is shaped to cooperate with the face 11 on the lower mold member to give the desired contour to the blank. 5

10 The wall 9 has a circumferentially extending opening 14 in its upper portion through which the container 1 may be inserted into the mold, and an annular shoulder 15 upon which the container 1 rests. The container is placed in the mold as 15 shown in Fig. 2, after which the upper and lower mold members 12 and 10 are brought together to the position shown in Fig. 3. The mold forms, in substance, a permanent part of a suitable press such as an hydraulic press, being fastened in the 20 press in any suitable manner. The press and the detail arrangement for operating the parts of the mold are not illustrated as this forms no part of my present invention. Any suitable structure of press may be used. The upper mold 25 member 12 forces the elements which go to make up the gear wheel blank out of the container 1 and such elements are compressed in the mold to provide a preform, as is indicated at 16 in Fig. 3. The preform 16 is then removed from the 30 mold. The elements of the preform as thus compressed are thoroughly stuck together by the adhesive so that the preform may be handled as a unit and the preform has the general contour of the completed gear wheel blank, but at this 35 time the adhesive is cured to only a slight extent. The preform 16 is now ready for its final pressing to shape and the complete curing of the adhesive. This may be done immediately after it comes from the preforming mold or it may be 40 done at any other suitable time as is found convenient in the process of manufacture.

When the preform is to be given its final molding operation, it is first warmed to remove any moisture which may have been left in it or which 45 it may have absorbed from the atmosphere, and to render the adhesive plastic. To accomplish this result, I have found that it is desirable to warm the preform for about twenty minutes in an oven at a temperature of the order of 95° to 50 125° C. The preform is then placed in a finishing or final mold and heat and pressure applied to bring the preform to its final shape and cure the adhesive. For this purpose I may use a steam heated mold located in a suitable hydraulic 55 press. Such a mold is indicated diagrammatically in Fig. 4 wherein 17 indicates the lower member of the mold and 18 the upper member of the mold. The construction and arrangement of the mold and the parts of the press are not 60 illustrated in detail, since the specific structure forms no part of the present invention and since any suitable type of heated mold to which pressure may be applied may be utilized. Such molds are well known in connection with the 65 manufacture of devices of the character described.

I find it advantageous to initially heat the preform so as to render the adhesive slightly plastic before it is placed in the finishing or final mold, 70 for this insures that as soon as the molds are brought together the material of the preform will flow readily so as to assume the shape of and completely fill the mold. This avoids the forming of pockets into which adhesive can flow. 75 For the final molding operation I have found

a pressure of the order of 2,000 to 3,000 pounds per square inch and a temperature of the order of 160° to 170° C. satisfactory, the pressing and heating taking place for a time of the order of twenty to forty minutes. 5

After the final pressing and heating operation in the finishing or final mold, the finished blank is removed and is ready for use. A finished blank is shown in Fig. 5 wherein 19 indicates the hub, 20 indicates the web and 21 indicates the rim. 10

In Figs. 6 to 8 inclusive, I have shown a modified form of my invention for use when the gear wheel blank is to comprise a rim made up of rings formed from woven textile material, and a web and hub formed from a material such as 15 loose cotton treated with an adhesive.

In Fig. 6, 22 indicates a container corresponding to the container 1 of Fig. 1, the container being of a size to hold the material 23 which is to form the hub and web of the gear wheel blank. 20 The material 23 is first weighed or measured and placed in the container 22 after which the ring or rings 24 which are to form the rim of the blank are placed on top of the container as shown. The container is then placed in a warming oven 25 and the material heated in a moist atmosphere after the manner already described. After being heated it is then placed in the forming mold and given an initial pressing to provide the preform. The forming mold is illustrated diagrammatically in Fig. 7 wherein 25 indicates the casting or shell of the mold, 26 indicates the lower mold member and 27 and 28 indicate the upper mold member which is made in two parts, part 27 being of a size to compress the rim of the 30 blank and the part 28 being of a size to compress the web and hub of the blank. The elements 23 and 24 are placed in the mold as is indicated in Fig. 7, after which the mold is closed as shown in Fig. 8 to compress the elements 23 and 24 to 40 produce the preform 29. This operation may be carried out after a manner corresponding to that already described in connection with Figs. 2 and 3 of the drawings. The preform is then removed from the forming mold and is ready for 45 the final pressing and curing operation which may be carried out after the manner described in connection with Fig. 4 of the drawings. Fig. 9 shows a completed gear wheel blank constructed in accordance with the modification illustrated in 50 Figs. 6 to 8.

By my improved method I effect a reduction in the labor cost of handling parts during the process of manufacture. By the former method utilizing hand molds, that is, separate molds in 55 which the elements forming the gear wheel were assembled, it was necessary for the workmen to handle these molds in assembling the elements therein, in putting the molds in the press, and in removing the molds from the press and the finished gear wheels from the molds. In one instance, the double hand molds used weighed forty-five pounds each, which meant the handling, in the course of an eight-hour shift, a total weight of the order of twenty-five tons of 60 steel. By the new method, the workman has to handle only the thin sheet metal containers in which the gear wheel elements are initially assembled, for as will be clear, in this case the mold forms, in substance, a part of the press as 65 distinguished from being a separate unit which is inserted in a press. I have found that the application of my invention in one instance has reduced the direct labor cost by an amount of 70 the order of twelve percent over a former hand 75

mold method of manufacture. At the same time, I have found that the use of molds which in substance form a part of the press, is not more expensive than the former hand molds.

5 My invention has a further advantage in that it provides for a visual inspection of each gear wheel during the process of manufacture, that is, a visual inspection of the preform, a thing not provided for in the case of hand molds. By 10 a visual inspection of the preform, any defects due to the assembling of the elements may be corrected if such as to permit of correction, or if not, then the preform may be discarded, thus avoiding the complete manufacture of a defective 15 gear wheel blank.

What I claim as new and desire to secure by Letters Patent of the United States, is:

1. The method of manufacturing bodies comprising a number of dissimilar elements formed 20 from spinnable textile fibers treated with uncured adhesive binder, which elements are to be assembled to form an irregular shaped body having thick and thin portions, which comprises assembling the elements in a relatively light 25 weight container and subjecting them to an initial heating to soften the adhesive, placing the elements in a forming mold in definite relation to give the desired shape and compressing them to cause the elements to adhere but without curing the adhesive, thereby providing a preform, and finally placing the preform in a mold and applying pressure and heat to bring the preform to its final shape and cure the adhesive.

2. The method of manufacturing bodies comprising a number of dissimilar elements formed 30 from spinnable textile fibers treated with uncured adhesive binder, which elements are to be assembled to form an irregular shaped body having thick and thin portions, which comprises giving 35 the elements an initial heating in the pres-

ence of steam to soften the adhesive, placing the elements in a forming mold in definite relation to give the desired shape and compressing them to cause them to adhere but without curing the adhesive, thereby providing a preform, and finally placing the preform in a mold and applying heat and pressure to bring the preform to its final shape and cure the adhesive.

3. The method of manufacturing bodies comprising 10 a number of dissimilar elements formed from spinnable textile fibres treated with uncured adhesive, which elements are to be assembled in definite relation relatively to each other and united to form a body, which comprises assembling the elements in a relatively light 15 weight container not adapted for compression of the elements therein, transferring the assembled parts from such container to a preforming mold and subjecting the parts to pressure to provide a preform, and placing the preform in a final 20 mold and applying pressure and heat to consolidate the structure and cure the adhesive.

4. The method of manufacturing bodies comprising a rim element and a rim connecting web 25 element formed of spinnable textile fibres treated with uncured adhesive binder, which elements are to be assembled to form an irregularly shaped body having a thick rim portion and a relatively thin web portion, which comprises assembling all the elements in the desired positions relatively 30 to each other in a preforming mold and subjecting them to heat and pressure in such mold to soften the adhesive and stick the several elements together to provide a preform, removing the preform as a unit from the preforming mold 35 and placing the preform in a finishing mold and subjecting it to heat and pressure to bring the preform to its final shape and cure the adhesive.

CLARENCE W. MANSUR. 40